

1

2,982,015

## METAL ARTICLES AND MATERIALS FOR MAKING SAME

James B. Russell, Davenport, Iowa, assignor to Kaiser Aluminum & Chemical Corporation, Oakland, Calif., a corporation of Delaware

No Drawing. Filed Feb. 25, 1957, Ser. No. 641,821

16 Claims. (Cl. 29—196.2)

This invention relates to composite metal articles having a ferrous metal base portion coated with a particular aluminum base alloy, the process for producing such composite articles and the aluminum base coating alloys. More particularly, the invention relates to aluminum alloys particularly adapted for the hot dip coating of a ferrous metal base, the hot dip process and the resulting composite metal article.

Coatings of aluminum on iron and steel products are highly desirable, since the composites resulting in effect embody the superior properties resident in each metal. To the strength and other desirable characteristics of the iron or steel core, the aluminum coating adds the more salient properties of resistance to corrosion and oxidation at both atmospheric and elevated temperatures, enhanced electrical conductivity, improvement in the facility of brazing and soldering of aluminum to steel, and a more attractive appearance.

As pointed out in my related copending applications S.N. 264,661, now abandoned, and S.N. 264,662, now Patent No. 2,782,493, directed to other particular aluminum base coating alloys and the composite metal articles produced therewith, it has been discovered that superior results may be obtained with certain aluminum base alloys as the coating material in regard to such factors as the appearance and continuity of the coating, and the ductility of the composite metal article compared with aluminum coated ferrous base composites utilizing high purity aluminum or commercially pure aluminum (2S alloy). With regard to the results obtained with aluminum base alloys of a given composition, the primary factor to be considered is the intended use or purpose of the composite article being produced. For example, in the fabrication of aluminum coated ferrous base metal products, it is often necessary that the composite article exhibit the ability to withstand high degrees of deformation upon subsequent working or forming. Such composite aluminum coated articles as wire or strip, which are usually subjected to continuous coating processes, and which are subsequently subjected to drawing or other forming operations must possess good ductility so that the coating will not crack and break away, that is, peel or flake off from the base metal during the subsequent working. In addition, the adherence of the aluminum coating to the ferrous metal base is involved in regard to the required characteristics that the coating will not peel or spall. Also freedom from tendency of the coating to crack during subsequent operations or in service is necessary so as to avoid any exposure of the base metal to corrosion. The combination of excellent ductility characteristics of the composite, and adherence of the coating together with excellent appearance of the coating is the objective attained with the particular aluminum base alloys to which the above referred to copending applications are directed.

In many instances, however, there are certain end uses or purposes for aluminum coated ferrous base metal articles in which ductility is relatively unimportant, and

2

appearance and continuity of the coating in regard to coverage, smoothness, texture, luster and other factors become of primary importance. For example, in the coating of rigid or semi-rigid articles such as castings and the like, wherein batch or semi-continuous processes of coating are in general employed, appearance and continuity of the coated composite are the foremost factors to be considered. Ductility is relatively unimportant since the article in its coated form is not subjected to any extensive deformation or subsequent working operations. Other specific examples of such articles are forgings, stampings and other shaped semi-finished or finished ferrous base articles.

Of the several processes for the production of aluminum coated ferrous base composite articles, the hot dip method is the most desirable from an economic standpoint and from the standpoint of range of applicability. However, the production of "aluminized" (aluminum-coated) ferrous base metal articles by means of the advantageous hot dip method, to which the present invention is particularly directed, has presented many problems. In regard to the hot dip process, other factors in addition to appearance and continuity of the coating and ductility of the composite are involved. These are primarily the molten bath operational characteristics, such as apparent fluidity, wettability of the ferrous base metal with the molten aluminum bath, forming rate, thickness and tenacity of the oxide film on the molten bath surface, which principally influence those characteristics of the coating determining appearance and continuity, such as coverage, smoothness, texture and luster, as well as adherence, in the as-coated condition.

As indicated in my copending applications above referred to, difficulty has been encountered in the use of high purity or commercially pure aluminum in the hot dip coating of ferrous metal articles in regard to the inability to obtain composite articles having the requisite ductility. This problem has been circumvented by the addition of certain alloying constituents which have effectively reduced the thickness and hardness of the intermetallic iron-aluminum layer which forms between the basis metal and the coating alloy. Thus, aluminum base alloys eminently suitable for coating wrought products such as wire and strip have been developed wherein the composite article produced may be subjected to subsequent forming operations without cracking or spalling of the aluminum base alloy coating. However, high purity or commercially pure aluminum as the coating materials for ferrous metal articles by the hot dip process also exhibit definite deficiencies in regard to the appearance of the coatings produced with respect to such factors affecting appearance as adherence, and continuity of the coating, smoothness, coverage, texture and even luster. In most instances the appearance of high purity is poor due to the large grains visible and a marked grain boundary depression in the surface. With commercially pure aluminum (2S alloy), the large grain structure tends to persist while the coatings are relatively dull due to an opaque oxide film. Also, particular difficulty has been encountered with hot dip coatings on castings wherein there has been a pronounced inability to produce coatings where coverage is complete, that is, continuity of the coating is lacking; and moreover the coatings are often of poor quality in regard to smoothness, texture and luster.

It is to this problem relating to the appearance and continuity of hot dip aluminum alloy coatings on ferrous base metal articles that the present invention is particularly directed.

It is, therefore, a primary purpose and object of the invention to provide hot dip aluminum alloy coated ferrous base metal articles which exhibit excellent appearance and continuity of the coatings in regard to coverage,

smoothness, texture and luster of the coatings and other factors affecting appearance.

It is a further object of the invention to provide particular aluminum base alloys adapted for the hot dip coating of ferrous base metals characterized by improved wettability of the ferrous metal base and their ability to form coatings and composite articles exhibiting excellent properties of adherence of the coating, and appearance and continuity of the coatings in regard to brightness, smoothness, coverage, and substantial absence of undesirable visible large grain surface effect.

It is a more specific object of the present invention to provide aluminum alloys for coating ferrous metal wherein the appearance and continuity factor including such properties as coverage, smoothness, texture and luster of the coating are of paramount importance and ductility of the composite is not a significant factor, which aluminum base coating alloys are superior in regard to the above-mentioned properties of the coating compared to high purity or commercially pure aluminum as a coating material.

It is a further object of the invention to provide a method of hot dip coating ferrous metal with particular aluminum base alloys to produce coatings on composite articles having the desirable combination of properties above-mentioned while operating at advantageous temperatures in regard to minimizing the thickness of the intermetallic alloy layer and without any substantial adverse effect on the operational characteristics of the molten coating metal.

A specific object is to provide particular aluminum base alloys as coating material for semi-rigid and rigid ferrous metal articles, such as castings, wherein excellent appearance of the coating is obtained in regard to the factors including adherence, coverage, smoothness, continuity, texture and luster thereof.

These and other objects and advantages of the invention will be apparent from the following detailed description thereof.

It has been discovered according to the invention that hot dip aluminum coatings on ferrous base metal of improved appearance in regard to coverage, continuity, smoothness, texture and luster compared to high purity aluminum and commercially pure aluminum are obtained by the utilization of certain ternary and more complex aluminum base alloys. These alloys, in addition, present an appearance of coating far superior to that provided by the known aluminum-silicon binary alloys, which as coating materials are effective to produce composite ferrous base articles of improved ductility.

In general, the aluminum base alloys of the invention contain small but effective amounts of chromium, and at least one of the elements molybdenum and tungsten, preferably only one of the last two named elements being utilized, to produce the above-mentioned desired results. It is to be noted that molybdenum is the preferred constituent to be added to the chromium-containing aluminum alloy, but that tungsten may be used more or less interchangeably therewith. It was found that the presence of chromium and molybdenum, or chromium and tungsten, notably the former two, provided distinct improvement in the coverage of the coating obtained on all types of ferrous bases. The coatings were continuous and smoother in surface texture in comparison with coatings produced by high purity aluminum and commercially pure aluminum (2S alloy). In addition, the chromium constituent of the aluminum base alloy coating increased the attractiveness of the color and luster of the coating in solid form on the ferrous base.

The coating alloys of the present invention provide remarkable results in regard to adherence, continuity, coverage and smoothness of coatings applied to cast ferrous metal articles—and are accordingly eminently suitable for utilization in the hot dip process wherein appearance is the primary factor and ductility of the com-

posite article produced is relatively unimportant. In regard to ductility, however, it must be noted that the alloys of the present invention produced composites which upon subjection to 180° flat bend tests and spiral wrap tests exhibited ductilities which were at least comparable to and in some cases better than the ductilities of composites utilizing high purity or commercially pure aluminum.

The elements chromium, molybdenum and tungsten generally may be present in amounts of from about 0.1 to about 0.40% each, the total not exceeding about 0.5%. The preferred range is from about 0.15 to about 0.25% each of these elements, and in general, as noted above, it is preferable to employ only chromium and molybdenum, or chromium and tungsten, and not all three of the elements, although the latter polynary alloy is definitely included within the scope of the invention, since, for example, lesser amounts of molybdenum may be employed and tungsten added to the chromium-molybdenum alloy, although when all three elements are present it is still preferred not to substantially exceed a total of about 0.5%.

As a further feature of the invention, it was discovered that the appearance of the above-defined ternary and more complex aluminum base alloys could be still further improved by the addition of at least one, and preferably only one, of the elements boron, titanium, vanadium and zirconium. Of these elements, titanium is the preferred species, although all of the named elements contribute to a marked improvement in the appearance of the coating alloys of the invention by markedly increasing the smoothness of the alloy coating and rendering the surface appearance more uniform and of even luster. In addition, an improvement in the ductility of the alloy coating was noted with small but effective additions of these elements. The visible grain, marring the appearance of high purity aluminum and 2S alloy coatings, was eliminated by the presence of one or more of these elements.

The element boron as one of the above group produces the advantages above noted, and, in addition, may be advantageously used to reduce bumpiness sometimes occurring in the coatings and to effect a general smoothing action on the coating.

Additions of boron and titanium are recommended in amount from about 0.02 to about 0.2% by weight of the alloy. The preferred range of these elements is from about .02 to .05% B and 0.02 to 0.1% Ti. When used together the preferred total is about 0.06%. The other two elements, namely vanadium and zirconium are recommended in amount from about 0.1 to about 0.25%. Although single additions of these elements are preferred, they may be used collectively, particularly where only two such elements are employed. In any event, the total where vanadium and zirconium are used collectively should not exceed about 0.5%.

It has also been found according to the invention that very limited or small amounts of beryllium have a desirable effect on the appearance of the coatings. This element exhibits the ability to reduce the amount of surface oxide on the molten aluminum alloy coating bath. The use of beryllium is particularly advantageous when coating with aluminum alloys containing silicon or sodium. Brown oxides are formed on the bath surface when these elements are incorporated in the molten coating alloy and cause staining of the coating. Amounts of from about 0.001 to 0.015% of beryllium are very effective in preventing the formation of this stain due to the brown oxide, and at the same time do not have any adverse effect on the ductility of the coating. A preferred lower amount of about 0.002% beryllium is recommended.

The use of beryllium in these amounts is to be distinguished from the use of beryllium in larger amounts where it functions similarly to silicon in having a pro-

nounced intermetallic layer thickness reducing effect. In any event, beryllium as an optional element in the coating alloys of the present invention for improvement in the appearance of the composite is limited to amounts below 0.02%, and amounts substantially in excess of this value are required to provide a decrease in the thickness of inter-metallic layer and resulting improvement ductility.

Where beryllium is added to the molten aluminum coating alloy bath, additions are made periodically to replace that lost through oxidation and due to chlorine fluxing, when the latter method is employed. These additions are made preferably by adding aluminum-5% beryllium hardener to maintain the composition at the desired beryllium content in the alloy.

It has been found that the alloys of the present invention may also advantageously contain an additional constituent, namely zinc, which contributes along with chromium and molybdenum to an increase in the surface brightness or luster of the coating and the attractive color thereof. In addition, the zinc constituent also contributed to an improvement in appearance of the coating by its beneficial effect on the continuity thereof. In general, additions of zinc in amounts from about 0.5 to about 2% by weight of the total alloy composition were found to be effective in this regard. The preferred range for zinc is from about 0.6 to about 1%, since in some instances coatings containing as high as 2% zinc exhibited a tendency toward a spangling effect on the surface of the coating, although the presence of one of the elements of the group including titanium set forth above had a definite counteracting effect in this regard. Amounts of zinc as high as 2% in some instances tended to decrease fluidity of the melt, although not to a disqualifying extent. The zinc constituent also appears to contribute to the cathodic protection of the ferrous base, particularly where the base would become exposed due to any cracking of the aluminum base, alloy coating during use of the composite article.

The alloying constituents of the present invention exerted a beneficial effect on the operational characteristics of the aluminum melt by improved wettability to the ferrous base. Further, they exerted no adverse effect in regard to such factors as apparent fluidity, oxide forming rate, oxide thickness and tenacity in the molten state. In fact, in certain instances the oxide forming rate, oxide thickness and oxide stain, the former characteristic judged qualitatively, were reduced by the presence of certain of the alloying constituents of the present invention, notably beryllium, as set forth above.

As examples of specific alloys which exhibited outstanding appearance in the as-coated condition relative to the reference alloys, namely 99.9% aluminum and commercially pure aluminum (2S alloy) the following may be mentioned: (1) 0.2% chromium-1% zinc-0.2% molybdenum-.07% titanium; (2) 0.2% chromium-0.2% molybdenum-0.06% titanium; (3) 0.2% chromium-0.2% molybdenum.

The aluminum alloys of the invention embrace those coating materials which may be designated as the ternary and more complex alloys set forth above wherein the balance of the alloy is substantially all aluminum and impurities in normal amounts. The term "impurities in normal amounts" as used herein and in the appended claims includes the iron which may be progressively picked up by the molten aluminum alloy bath from the ferrous base during continued operation, as discussed hereinbelow. Other elements in the form of residuals such as silicon, and copper may be present in normal impurity amounts without unduly adversely affecting the beneficial results obtained by the alloying constituents of the invention with the aluminum coating metal.

The aluminum base alloys may be prepared by adding the addition elements to the molten aluminum bath in ele-

mental form or in suitable compound form. Preferably, however, the desired amounts of the elements are added to the bath in the form of master alloys of aluminum, for example, Al-2% Cr, Al-2.5% Mo, Al-2% Zr, etc. Zinc, however, is most conveniently incorporated by direct addition to the bath as elemental zinc. Of course, these alloys or "hardeners" may be previously prepared and then remelted to form the coating bath with proper dilution with aluminum.

In utilizing the alloys of the present invention in the hot dip process various procedural modifications may be employed. However, since these alloys are particularly intended for utilization in coating ferrous metal articles wherein the composites produced are more or less semi-finished or finished articles, the process most advantageously employed is the batch or semi-continuous process. Of course, the invention is not to be regarded as limited to the particular manner in which the aluminum alloy coating is applied to the ferrous base by the hot dip method and in many instances the continuous process may be employed for coating wire and strip materials wherein ductilities comparable to those of high purity and commercially pure aluminum coated composites are acceptable. In either case, the coating alloys and molten baths prepared therefrom produce aluminum alloy coated ferrous metal articles superior in appearance and continuity to similar articles coated with high purity aluminum and commercially pure aluminum, and far superior to articles produced by the utilization of aluminum-silicon binary alloy coating materials.

The ferrous articles to be coated are first thoroughly cleaned by any suitable method, such as acid pickling to remove oxide film or scale unless the surface condition renders this treatment unnecessary. They may then be rinsed and dried, and immersed in the coating bath with or without the use of a conventional flux. On the other hand, the articles with or without pickling depending upon the nature of the surface may be pretreated by bright annealing in suitable apparatus in an inert or reducing atmosphere and then directly immersed in the molten coating bath without exposure to the atmosphere.

The bath temperature is maintained sufficiently high so that the alloys employed are completely molten. Of course, the particular bath temperature depends upon the coating alloy composition and the composition and nature of the ferrous article; and in regard to the alloys herein disclosed temperatures of from about 1250 to about 1375° F. are recommended. Since thickness of the Fe-Al interfacial layer increases with bath temperature, it is recommended that the lowest operating temperature consistent with good coating results be used.

The time of immersion depends principally upon the composition of the molten bath, the composition and nature of the ferrous article, and the temperature of the molten bath. The immersion time and also the bath temperature may be regulated to produce a composite most suitable for the intended application. Extending the time of immersion tends to increase the thickness of the Fe-Al layer and accordingly the shortest immersion times consistent with satisfactory coverage are usually recommended.

#### Example

As an example of one specific procedure in utilizing the coating materials of the invention to produce composites by the hot dip method, the following is set forth as illustrative without constituting a limitation on the scope of the disclosure and claims appended hereto:

Specimens consisting of mild steel strip containing 0.2% manganese and less than 0.1% carbon, 12 inches in length, .25 inch wide and .036 inch thick were used. All specimens were degreased with carbon tetrachloride and wiped dry with cloth, then pickled in a 40% HCl solution for from 15 to 25 seconds at a temperature of 140-

160° F. This was followed by a water rinse and the cleaned specimens were dried with gauze.

The specimens were then dipped in a molten bath of aluminum base alloy containing 0.2% chromium-0.2% molybdenum and 0.06% titanium, the balance aluminum and less than 1% normal impurities. Identical specimens were dipped in molten baths of 99.9% aluminum, commercially pure aluminum (2S alloy) and a 5% silicon-aluminum binary alloy. No fluxes were employed, and the specimens were immersed for from 15 to 30 seconds with the bath temperature maintained at about 1300° F. The coated specimens were withdrawn and tapped lightly while in a vertical position to facilitate removal of excess coating.

The surfaces of the specimen coated with 99.9% aluminum were mottled in appearance due to the visible large grain structure of the coating and the coverage of the coating at the edges of the strip tended to be incomplete, or where continuous it was rough.

The coating of commercially pure aluminum (2S alloy) was also characterized by a visible large grain, which, however was somewhat obscured by a more or less opaque oxide film which presented a relatively dull appearance compared to a metallic luster. The coating on the edges of the strip was rough and continuity was slightly lacking.

The 5% silicon-aluminum alloy coating had a dull greyish color seriously lacking in luster, and was characterized by a markedly rough surface texture over substantially the whole strip, although the coating was continuous on the strip edges.

The strip coated with the alloy of the invention had a uniform, pleasing luster and was exceptionally smooth in texture with complete coverage even at the edges. No objectionable large grain was visible on the surface of the coating.

Accordingly, the alloys of the invention as coating materials for ferrous base metals produce composites of improved appearance and continuity as evidenced by the excellent coverage, smooth grainless texture and luster of the coatings compared to conventional high purity and commercially pure aluminum coatings, and vastly improved appearance as contrasted with the aluminum-silicon alloys.

It is to be noted that during the course of continued operation either on the batch or continuous basis, the molten aluminum alloy bath gradually increases in iron content due to pickup by dissolution of iron from the basis metal. Small amounts of iron in the coating alloy, up to just below saturation, for example, 2.5% at the usual coating temperatures, may be tolerated without any significant adverse effect on the character of the coating and composite. However, when the iron content increases to, for example 3 or 4%, it exceeds the saturation point (on the liquidus line) depending upon the particular coating temperature and composition of the bath, and begins to affect quality of the coatings and composites, particularly in regard to smoothness. Various procedures may be adopted for reducing the iron content and increasing effective bath life among which may be mentioned discontinuance of operation of the bath while permitting the heavy iron component to settle out of the molten aluminum alloy, or addition of fresh amounts of uncontaminated aluminum alloy to effectively reduce the concentration of iron in the total molten bath. Of course, employing a new bath of aluminum alloy obviates the problem, but is a less desirable solution with regard to treating a maximum amount of ferrous base metal with a minimum aluminum alloy consumption.

All percentages in the claims are by weight of the total alloy.

This application is a continuation-in-part of my pending application S.N. 261,746, filed December 14, 1951, now abandoned.

What is claimed is:

1. A composite article comprising a base portion of ferrous metal hot dip coated with an aluminum base alloy of improved wettability to the ferrous base consisting essentially of chromium in amount from about 0.1 to 0.4%, and at least one of the elements molybdenum and tungsten in amount from about 0.1 to 0.4%, the total amount of these alloying constituents not exceeding about 0.5%, the balance substantially all aluminum and impurities in normal amounts.
2. A composite article according to claim 1 in which the aluminum base alloy contains also at least one element selected from the group consisting of boron, titanium, vanadium and zirconium in amounts from about 0.02 to about 0.2% boron and titanium, and about 0.1 to about 0.25% vanadium and zirconium, the total of these elements not exceeding about 0.5%.
3. A composite article according to claim 1 in which the aluminum alloy also contains zinc in amount from about 0.5 to about 2%.
4. A composite article according to claim 1 in which the aluminum alloy also contains from 0.001 to below 0.02% beryllium.
5. A composite article according to claim 2 in which the aluminum alloy also contains from 0.001 to below 0.02% beryllium.
6. A composite article according to claim 3 in which the aluminum alloy also contains from 0.001 to below 0.02% beryllium.
7. A composite article according to claim 3 in which the aluminum base alloy contains also at least one element selected from the group consisting of boron, titanium, vanadium and zirconium in amounts from about 0.02 to about 0.2% boron and titanium, the total of boron and titanium not exceeding about 0.06%, and about 0.1 to about 0.25% vanadium and zirconium, the total of vanadium and zirconium not exceeding about 0.5%.
8. A composite article according to claim 7 in which the aluminum alloy also contains from 0.001 to below 0.02% beryllium.
9. A hot dip coated product comprising a ferrous metal base coated with an aluminum base alloy consisting essentially of from about 0.15 to about 0.25% chromium, and one element selected from the group consisting of molybdenum and tungsten in amount from about 0.15 to about 0.25%, balance substantially all aluminum and impurities in normal amounts.
10. A composite article according to claim 9 in which the aluminum base alloy contains also one element selected from the group consisting of boron, titanium, vanadium and zirconium in amounts from about 0.02 to about 0.05% boron, from about .02 to 0.1% titanium and about 0.1 to about 0.25% vanadium and zirconium.
11. A composite article according to claim 9 in which the aluminum alloy also contains from 0.002 to 0.015% from about 0.6 to about 1%.
12. A composite article according to claim 9 in which the aluminum alloy also contains from 0.002 to 0.015% beryllium.
13. A composite article according to claim 10 in which the aluminum alloy also contains from 0.002 to 0.015% beryllium.
14. A composite article according to claim 11 in which the aluminum alloy also contains from 0.002 to 0.015% beryllium.
15. A composite article according to claim 11 in which the aluminum base alloy contains also one element selected from the group consisting of boron, titanium, vanadium and zirconium in amounts from about 0.02 to about 0.05% boron, from about .05 to 0.1% titanium and about 0.1 to about 0.25% vanadium and zirconium.
16. A composite article according to claim 15 in which the coating alloy contains from 0.002 to 0.015% beryllium.

References Cited in the file of this patent  
UNITED STATES PATENTS

|           |           |               |
|-----------|-----------|---------------|
| 1,663,150 | Archer    | Mar. 20, 1928 |
| 1,850,355 | Russell   | Mar. 22, 1932 |
| 2,091,419 | Schroeder | Aug. 31, 1937 |

|           |
|-----------|
| 2,280,174 |
| 2,357,450 |

|         |               |
|---------|---------------|
| Stroup  | Apr. 21, 1942 |
| Bonsack | Sept. 5, 1944 |

## OTHER REFERENCES

"Effect of Bath Composition Coating on Steel," Gittings et al., preprint published October 1950, ASM, 19 pages.

UNITED STATES PATENT OFFICE  
CERTIFICATE OF CORRECTION

Patent No. 2,982,015

May 2, 1961

James B. Russell

It is hereby certified that error appears in the above numbered patent requiring correction and that the said Letters Patent should read as corrected below.

Column 5, line 7, after "improvement" insert -- in --; line 46, for "fast" read -- fact --; column 8, line 55, after "aluminum" insert -- base --; line 55, for "from 0.002 to 0.015%" read -- zinc in amounts --.

Signed and sealed this 17th day of October 1961.

(SEAL)

Attest:

ERNEST W. SWIDER

Attesting Officer

DAVID L. LADD

Commissioner of Patents  
USCOMM-DC